

## 1

2,706,679

### LITHIUM HALIDE FLUX FOR TREATING MAGNESIUM-LITHIUM ALLOYS

Paul D. Frost, Columbus, Ohio, assignor, by mesne assignments, to Olin Mathieson Chemical Corporation, a corporation of Virginia

No Drawing. Application June 30, 1948,  
Serial No. 36,292

1 Claim. (Cl. 75—67)

This invention relates to fluxes for the treatment of magnesium alloys and provides an improved flux for use in melting magnesium-lithium base alloys, especially those containing appreciable amounts of heavy alloying elements.

A melting flux effectively used for magnesium-lithium base alloys has been described in a patent application of Alfred H. Hesse, entitled "Fluxes," Serial No. 603,749, filed July 7, 1945, now Patent No. 2,507,713 and comprises from 60% to 98% of a chloride component and from 40% to 2% of a fluoride component, said chloride component consisting of from 0 to 50% of potassium chloride, from 0 to 10% of alkaline earth metal chloride and the balance lithium chloride and said fluoride component consisting of at least one fluoride of the group consisting of potassium fluoride, lithium fluoride and alkaline earth metal fluoride, the total of the alkaline earth metal chloride and fluoride being less than 15% of the flux, said flux as initially used being practically free of sodium. This flux is especially useful with alloys whose specific gravity in the solid state is around 1.5 and is satisfactory for nearly all Mg-Li alloys. Ordinarily, the LiCl-LiF flux, being heavier than the Mg-Li alloys, remains for the most part below the melt with a thin film of flux covering the top of the melt and protecting it from reactive gases. However, certain recently developed high-strength alloys contain heavy alloying elements and have specific gravities of the order of 1.66 to 1.70, and in melting some of these heavier alloys, it has

## 2

been found difficult to obtain good separation of the flux from the metal during pouring. Therefore, it is desirable in some cases to increase the specific gravity of the flux. This has been done recently by adding BaCl<sub>2</sub> to the flux before pouring. However, it has now been found that BaCl<sub>2</sub> is undesirable because it is likely to break down and contaminate the Mg-Li alloys with metallic barium.

I have confirmed my conception that LiBr is an effective addition salt to increase the specific gravity of the LiCl-LiF flux. In accordance with my invention, I substitute LiBr for a major part of the LiCl and the LiF of the fluxes of the type described in said application. Previous investigation had shown that a eutectic existed at 15 about 75% LiBr-25% LiCl and that this eutectic melted at about 970° F. It has now been found that the melting point can be reduced to about 825° F. by the addition of 10% LiF. The combination of around 3 parts LiBr, 1 part LiCl, plus about 10% LiF has been used as a melting flux with heats of magnesium-lithium base alloys and found to be extremely fluid (because of its low melting temperature), during the first part of the melt, but to thicken considerably before pouring. The experimental heats were carried out with alloys comprising 6 Mg/Li, 25 16% Cd, 5% Ag. The theoretical density of the 3 LiBr/LiCl-10% LiF flux is about 2.93 g./cc. (solid) as against about 2.18 g./cc. for a 75% LiCl-25% LiF flux. A preferred flux would have a density somewhere between the two values.

30 A flux consisting of 75% LiBr-25% LiCl has also been tried and observed to act in a manner similar to the LiBr-LiCl-LiF flux. In several cases some burning was noted and it is believed that the density of the flux had been increased too much by the inclusion of too 35 great a proportion of LiBr. Experimental results definitely show that the melted alloys can be poured or cast without difficulties caused by poor separation between the flux and the alloy.

I claim:

40 A flux for the treatment of molten magnesium-lithium base alloys consisting of about 3 parts LiBr, 1 part LiCl and about 10% LiF.

No references cited.